

Aug. 16, 1955

E. S. PETTYJOHN ET AL

2,715,573

METHOD FOR GASIFYING COAL

Filed May 27, 1950

2 Sheets-Sheet 1



Inventors  
Elmore S. Pettyjohn  
Claus G. Von Fredersdorff  
By Bair, Freeman & Molinare  
Attest.

Aug. 16, 1955

E. S. PETTYJOHN ET AL  
METHOD FOR GASIFYING COAL

2,715,573

Filed May 27, 1950

2 Sheets-Sheet 2

Fig. 6



Fig. 7



Inventors  
Elmore S. Pettyjohn  
Claus G. Von Fredersdorff  
By Bair, Freeman & Molinare  
H. C. J. S.

1

2,715,573

**METHOD FOR GASIFYING COAL**

Elmore S. Pettyjohn, Evanston, and Claus G. von Fredersdorf, Roselle, Ill., assignors to The Institute of Gas Technology, Chicago, Ill., a corporation of Illinois

Application May 27, 1959, Serial No. 164,692

6 Claims. (Cl. 48—206)

This invention relates to a method and apparatus for preparation of calorific gases by the gasification of finely subdivided coal suspended in a flowing gas.

An object of this invention is to provide method and apparatus of the nature indicated capable of efficiently utilizing coal of high ash content to gasify such coal continuously and with a high output of calorific make gas per unit of apparatus space.

Other and further objects and features of the present invention will become apparent from the following description and appended claims as illustrated by the accompanying drawings showing, diagrammatically and by way of examples, apparatus according to the present invention. More particularly:

Figure 1 is a side view of an apparatus according to the present invention;

Figure 2 is another side view of the apparatus of Figure 1;

Figure 3 is a plan view of the apparatus of Figure 1;

Figure 4 is a fragmentary view similar to Figure 2 but showing a modification of the apparatus of Figures 1 to 3;

Figure 5 is a view similar to Figure 1 but showing still another modification of the apparatus of Figures 1 to 3;

Figure 6 is a side elevation, with parts shown in vertical section along the line 6—6 of Figure 7, and showing another apparatus according to the present invention; and

Figure 7 is a sectional view taken along the line 7—7 of Figure 6.

When proceeding according to the present invention, finely subdivided coal is suspended in flowing oxygen enriched air. Combustion of the coal is brought about and a temperature is maintained at which the ash content of the coal is slagged and at which carbon monoxide rather than carbon dioxide is generated. The temperature may be raised to a point where steam may be added to the suspension for bringing about a blue gas reaction.

From a practical operating standpoint, the characteristics in terms of which such a process may be evaluated including the following:

1. Calorific value of make gas
2. Completeness of coal gasification
3. Completeness of recovery of heat content of coal ("thermal efficiency")
4. Amount of gas generated per unit of apparatus space
5. Ease and completeness of ash separation
6. Minimum wear and erosion of apparatus

Items 1, 5 and 6 are believed to be self-explanatory. By the term "completeness of coal gasification" is meant simply the extent to which the coal is gasified or conversely the amount of coal still left in unburned form after passing through the gasification apparatus, no distinction being made on the basis of the calorific value of the gas produced. By the term "thermal efficiency" is meant the amount of heat available by combustion of a given amount of make gas cooled to room temperature

2

as compared with the heat available by combustion of the amount of coal fed into the apparatus in the manufacture of said amount of make gas.

From a cost standpoint, it is also important to know the amount of heat required (if any) in excess of that derived by combustion of coal being gasified and the amount of oxygen consumed for enriching the air in which the coal is suspended for gasification.

The operating variables which are controlled according to the present invention including the following:

1. The ratio of total gaseous oxygen added per unit weight of coal
2. Inlet oxygen concentration of the air-oxygen portion of the gaseous suspension medium
3. The ratio of steam (if any) to unit weight of coal
4. Rate and nature of gas flow through the apparatus
5. Residence time of gases in apparatus
6. Particle size of coal
7. Temperature of material entering the apparatus
8. Pressure

The above-tabulated operating variables, according to the present invention, are adjusted to maintain, among other things, a temperature high enough to cause slagging of the ash content of the coal and to cause a coal gasification yielding a maximum amount of carbon monoxide and a minimum amount of carbon dioxide. According to specific methods within the scope of this invention the temperature is maintained high enough to bring about a reaction with added steam.

20 The fusion temperature of the coal ash depends somewhat on the particular coal being gasified but generally ranges upwardly from about 2200° F. Thus, for practical purposes at least this temperature must be reached and maintained until the slag has been separated from the make gas. Separation of the coal ash from the make gas by slagging is an essential feature of the present invention. However, for other reasons, the operating temperature is in all cases maintained, in at least at one stage in the gasification process, at a temperature in excess of 2200° F., as explained hereinbelow. Nevertheless, even when such a higher temperature is generated and maintained at some stage ahead of the separation of ash, the temperature must not be permitted to fall to 2200° F. (or to the solidification temperature of the ash) until after the ash has been separated.

In the gasification of coal according to the present invention, the combustion of the coal apparently proceeds in two stages. First, the carbonaceous material in the coal is oxidized to carbon dioxide and next the carbon dioxide is reduced to carbon monoxide by residual carbonaceous material. At a temperature in excess of 2300° F. this second stage (reduction of dioxide to monoxide) approaches completion yielding a make gas containing relatively small amounts of carbon dioxide. Hence, the temperature is maintained about 2300° F. at least until this second stage of the combustion has been completed.

At temperatures ranging from 2500 to 3000° F., we can add steam, in amounts ranging up to 1 lb. of steam for each pound of coal, to form hydrogen and carbon dioxide by reactions involving steam and carbon monoxide and steam and carbon.

At temperatures of 3000° F. or higher, we find it possible to carry out both an incomplete combustion of part of the coal yielding principally carbon monoxide and a concurrent blue gas reaction with steam and the rest of the coal yielding both carbon monoxide and hydrogen.

For maintaining the indicated temperature range, an amount of heat must be generated in and/or carried into the gasification chamber equal to the heat losses occurring at this temperature range. The heat losses in question include the heat loss due to radiation and

convection; heat lost as sensible heat of make gas; and heat lost due to the more or less endothermic nature of a gasifying reaction, as when steam is used. The heat loss due to radiation and convection is best indicated in terms of amount of heat lost per unit of coal introduced into the apparatus. The loss of a given amount of heat per unit of time will be more or less significant depending on the amount of coal fed into the apparatus during this unit of time.

The heat lost as sensible heat of make gas will vary according to the amount and composition of the make gas produced. For instance, the nitrogen, steam and other non-calorific gas contents of the make gas will affect the amount of heat lost as sensible heat of make gas.

The amount of heat generated in the gasifying chamber (when the carbonaceous material in the coal is burned to carbon monoxide) depends, among other things, upon the completeness of the combustion of this coal or conversely upon how much of this coal passes through the apparatus without being burned.

Two of the operating variables controlled for effecting combustion of a maximum amount of the coal fed into the gasifying chamber are the particle size of the coal and the mixing of the coal with the gases entering the apparatus. We feed the coal into the apparatus in finely subdivided form. At least 80% of the coal passes a 100 mesh screen and at least 50% passes a 200 mesh screen. Preferably, practically all the coal passes through a 100 mesh screen and at least 50% passes through a 325 mesh screen. This finely subdivided coal is suspended in air or oxygen enriched air and injected tangentially at a rapid rate into a cylindrical chamber wherein vertical gas movement is effected. Additionally, oxygen enriched air or oxygen and, optionally, steam, are also tangentially injected into the vortex chamber. Thus, rapid and complete intermixing of reactants is assured in the rapidly flowing gaseous coal suspension. The latter may then be tangentially injected into a second vortex chamber where combustion and gasification take place. Additional amounts of air or oxygen enriched air may be injected tangentially into the second vortex chamber. Due to the fine particle size of the coal and its intimate intermixture with the suspending gases, the coal is quickly raised to combustion temperature and burned or gasified rapidly and completely in the second vortex chamber. In other words, the amount of coal passing through the apparatus without being burned is very small.

It should be noted, in this connection, that the above-disclosed fine particle size of the coal and the intimate intermixture of the coal with the reacting gases not only promotes more rapid and complete combustion and gasification of the coal, but also brings about the production of a make gas having a high ratio of carbon monoxide to carbon dioxide and therefore characterized by a relatively high calorific value.

Other operating variables that are controlled for maintaining the high temperature include the residence time of the coal suspension and of the gas formed therefrom within the apparatus and the pressure maintained in the apparatus. As the weight rate of flow through the apparatus is increased, thus shortening the residence time, the heat losses per weight unit of coal due to radiation and convection are lessened. A lower limit for the residence time is set by the time required for gasification of the coal with formation of carbon monoxide. The residence time is closely correlated with the pressure within the apparatus. Raising the pressure to superatmospheric levels increases the residence time, for at such increased pressures more weight units of gas are contained in each space unit of the apparatus, the volume of each weight unit of gas being inversely proportional to the pressure.

A temperature of from 2300° to 2500° F. can be maintained by feeding coal of the indicated fineness, effecting intimate coal-gas mixing, adjusting the residence time

to about 0.2 to 3.5 seconds and maintaining the apparatus at atmospheric or higher pressure, preferably at from 5 to 7 atmospheres. To raise the temperature to or above 2300° F., and to generate gas efficiently that has a heating value in excess of 100 B. t. u., the oxygen containing gas must contain more than 30% free oxygen and may contain as much as 98% oxygen. An oxygen content of 60% or more is preferred as giving the best results. The ratios of total oxygen to coal are disclosed hereinbelow. If a blue gas reaction is to be effected (at 3000° F. or higher) then the steam must be pre-heated at least to 2000° F. and preferably to 2200° F.

While the operating variables must be adjusted to maintain the above-indicated temperature range, the operating variables may be further adjusted while maintaining said temperature range to secure various types of results, as disclosed hereinbelow.

At temperatures below 3000° F. a relatively high ratio of oxygen to coal favors more complete coal gasification at the expense of the calorific value of the make gas and at the expense of thermal efficiency. Conversely, a relatively low ratio of oxygen to coal favors the formation of make gas of relatively high calorific value with high thermal efficiency but the coal is gasified less completely. We have found further that as the oxygen concentration in the suspending gas is increased, the ratios of oxygen to coal favoring either more complete coal gasification or formation of make gas of relatively high calorific value with high thermal efficiency are both increased. Some thermal efficiency and calorific value of make gas may be sacrificed to secure more complete coal gasification, and vice versa. The specific gravity and the carbon monoxide to hydrogen ratio in the make gas can both be lowered by the use of steam up to about 0.5 to 1.0 pound per pound of coal.

At temperatures in excess of 3000° F., and when both steam and oxygen-containing gas are caused to react with the coal, maximum thermal efficiency, maximum calorific value of make gas and maximum coal gasification may be effected at about the same ratio of oxygen to coal.

In general, the total gaseous oxygen to coal ratio should be maintained within ranges depending on the inlet oxygen concentration and tabulated as follows:

|                              | Inlet oxygen concentration in percent |         |         |         |         |
|------------------------------|---------------------------------------|---------|---------|---------|---------|
|                              | 30                                    | 60      | 70      | 90      | 98      |
| lb. O <sub>2</sub> /lb. coal | 0.5-0.9                               | 0.6-0.9 | 0.6-0.9 | 0.7-0.9 | 0.7-1.0 |

The above-described methods may be practiced in apparatus shown in the accompanying drawings and described as follows:

In Figures 1 to 3 the reference numeral 10 indicates generally a gas-making apparatus constructed of suitable refractory material. Within the apparatus 10, there is defined a generally cylindrical vortex chamber 12 having a horizontal axis. A suspension of finely divided coal in a gas enters the vortex chamber 12 through a generally tangential conduit 14. Steam or other gas is injected into the vortex chamber 12 through a second generally tangential conduit 16 spaced from the conduit 14 by about 90°. Gas is discharged from the vortex chamber 12 through a central axial discharge conduit 18 opening tangentially into a generally vertical cylindrical gasification chamber 20 provided near its bottom with a slag outlet 22 and a gas outlet 24. The latter is arranged at a slightly higher level than the slag outlet 22 to prevent blocking by slag. Additional air or oxygen enriched air may be injected tangentially into the gasification chamber 20 through a conduit 26.

In the operation of the apparatus of Figures 1 to 3 a suspension of finely divided coal in air, oxygen enriched air or oxygen and, if desired, some steam enters the vortex chamber 12 through the conduit 14. The latter is

disposed so that the injected suspension will have an unobstructed passage until the suspension impinges against the steam issuing into the vortex chamber 12 from the conduit 16. The steam thus functions as a protective blanket to prevent erosion of the wall of the vortex chamber 12 at the area where otherwise the coal suspension would impinge directly against the wall of the vortex chamber. The suspension of coal in the two gases injected through the conduits 14 and 16 will flow vertically within the chamber 12 whereby intimate mixing and selective grinding of relatively coarse coal particles will be effected. The resulting uniformity of particle size is an advantage for in the subsequent gasification coal particles of about the same particle size will be gasified more uniformly. The suspension of uniformly sized particles in the gaseous mixture passes through the conduit 18 tangentially into the gasifying chamber 20 where gasification takes place, secondary air or oxygen enriched air being preferably injected through the conduit 26. The gas flow within the chamber 20 is vertical so that molten slag will collect on the inside walls and flow down to the bottom of the chamber 20 where accumulated slag may be removed in molten form through the conduit 22. The make gas is collected through the conduit 24.

In any process where coal particles are raised to a temperature above the coking or fusion range, the hot coal particles tend to coke and agglomerate and to be deposited as adherent masses on the walls of the apparatus which interfere with the operation of the apparatus and are difficult to remove. Further, in any process where a slagging temperature is reached, the molten slag tends to accumulate on the walls of the apparatus, entrapping coal particles and easily forming viscous masses that may block the apparatus.

In our process the coal particles are very rapidly heated to a coking or fusion temperature, but deposition of the coal particles immediately after injection is prevented by the above-mentioned protective blanket of steam. Past this point the coal particles are suspended and carried by vertically flowing gas and the volatile content of the coal is volatilized very rapidly so that the coal is partially devolatilized before again being thrown into contact with a solid surface. When a slagging temperature has been reached in the gasifying chamber 20, the slag will collect on the walls of the apparatus due to the vertical movement of a suspending fluid and then flow downwardly to be collected at the bottom of the chamber 20.

A modification of the apparatus of Figures 1 to 3 is shown in Figure 4 when the conduit 14 is constricted as at 15, to form a restricted throat or orifice. If an entrainment of coarsely granular coal in a gas is caused to pass through the conduit 14, the coal granules being small enough to pass freely through the constriction 15 and if on such passage a pressure drop of at least 15 pounds per square inch is effected with acceleration of the entraining gas, then the coal granules will be shattered on passing through the constriction 15. Reference is made to the copending applications of John I. Yellott, Serial Nos. 22,154 and 762,589, filed, respectively, April 20, 1948, and July 22, 1947 (now Patents No. 2,515,542 and No. 2,515,541, respectively), for a detailed description of such means and methods for comminution of coal and the like.

Figure 5 shows apparatus generally similar to that of Figures 1 to 3, except for the fact that the gas flow through the gasifying chamber takes place in an upward direction. As shown, the apparatus of Figure 5 generally indicated at 30 and constructed of suitable refractory material includes a vortex chamber 32 of cylindrical shape and having an axis extending generally horizontally. A suspension of coal in a gas is injected tangentially into the vortex chamber 32 through a conduit 34 while a blanketing gas is injected tangentially into the vortex chamber through a conduit 36. An axial central dis-

charge aperture 38 affords communication between the vortex chamber 32 and the bottom portion of the vertical gasifying chamber 40 from which molten slag may be discharged through a conduit 42 having an inner opening below that of conduit 38. Additional air or oxygen enriched air may be tangentially injected into the gasifying chamber 40 through a conduit 44. Make gas produced in the chamber 40 may be collected through a conduit 46.

While the apparatus of Figure 5 functions similarly to that of Figures 1 to 3, it may be noted that, since in both gasifying chambers 20 and 40 maximum temperature is reached adjacent the discharge openings of the conduits 18 and 38, the maximum temperature in the case of the apparatus of Figures 3 and 5 will be reached immediately above the layer of molten slag collecting on the bottom of the chamber 40 so that as a result, this slag will be less viscous.

Both the apparatus of Figures 1 and 3 and that of Figure 5 are suitable for operation at any temperature in excess of 2300° F. Figures 6 and 7, on the other hand, show apparatus especially designed for operation at temperatures of 3000° F. or higher. More particularly, the apparatus of Figures 6 and 7 includes a heat exchange device for recovering the heat of the make gas produced for utilizing this recovered heat to superheat steam to 2000° F. or higher.

The apparatus of Figures 6 and 7 includes a cylindrical vortex chamber 50 having a vertical axis into which a suspension of coal in air, oxygen enriched air, steam or mixtures thereof is tangentially injected through a conduit 52. Preheated steam at a temperature of 2000° F. or higher is injected tangentially through a conduit 54. The vertically flowing coal suspension is discharged centrally and axially from the vortex chamber 50 directly into a vertically arranged tubular gasifying chamber 56 having, at its bottom, a slag outlet 58 and, provided at a slightly higher level, with a hot make gas discharge conduit 60. Additional preheated air or oxygen enriched air may be injected into the gasifying chamber 56 through a conduit 62.

The hot make gas is discharged through conduit 60 into the bottom of a fluidizing vessel 64 containing a solid more or less finely subdivided heat exchange medium 66. The hot make gas flows upwardly through the vessel 64 and the heat exchange medium contained therein and passes through a gas-solid separator 68 into a discharge conduit 70. The heated heat exchange medium 66 overflows through a conduit 72 into a steam conduit 74 where the heat exchange medium is picked up by steam to be superheated (which may contain added air or oxygen enriched air) and carried by the steam into an upper fluidizing vessel 76. There heat exchange between the steam and the heat exchange medium is completed. The resulting superheated steam passes through a gas-solid separator 78 into the conduit 54 while the heat exchange medium flows through a conduit 80 back to the lower fluidizing vessel 64 for reheating by further amounts of hot make gas.

The temperature in vortex chamber 50 receiving the coal suspension and superheated steam is upwardly of 3000° F. At the slag discharge conduit 58, the temperature in the gasifying chamber 56 is at least 2500° F. The steam is superheated in the fluidizing vessel 76 to 2000° F. or higher.

As in the apparatus of Figures 1 to 5, provision is made for a protective steam blanket to prevent erosion of the apparatus by impingement of the injected coal suspension. Likewise, intimate admixture of steam and coal suspension and selective grinding of the coarser coal particles will be effected in the vortex chamber 50.

In general, the coal suspension is injected into the apparatus of Figures 1 to 7 at a velocity of at least 150 to 200 feet per second and is thereafter caused to flow through the apparatus at least 100 feet per second.

We give hereinbelow operating results obtained using

the above-described method and apparatus. These results are obtained by averaging the results obtained in the gasification of a coal (Hawthorne Mine #6 Seam, Illinois-type high volatile C bituminous) having a proximate analysis of 3.5% moisture, 32.7% volatile matter, 51.7% fixed carbon and 12.6% ash. The ultimate analysis was 65.40% carbon, 4.73% hydrogen, 1.70% nitrogen, 11.23% oxygen, 3.94% sulphur and 13.00% ash. The ash was completely fluid at 2282° F. The coal was further characterized by a gross heating value (dried) of 11,840 B. t. u. per pound. The particle size of the coal is tabulated as follows:

| U. S. Sieve            | 40 | 60 | 100 | 200 | 325 | -325 | 15 |
|------------------------|----|----|-----|-----|-----|------|----|
| Weight Percent Passing | 1  | 3  | 10  | 35  | 21  | 30   |    |

Results obtained in the apparatus of Figures 1 to 3 and 5 at atmospheric pressure and at a steam temperature not in excess of 900° F. are tabulated as follows:

| Exp. No. | Lb. Steam/<br>Lb. Coal | Lb. O <sub>2</sub> /<br>Lb. Coal | Percent<br>O <sub>2</sub> Conc. | Percent<br>Coal<br>Gasified | Thermal<br>Eff. | B. t. u.,<br>Cu. Ft. |    |
|----------|------------------------|----------------------------------|---------------------------------|-----------------------------|-----------------|----------------------|----|
| 1        | 0.46                   | 1.06                             | 70.0                            | 85.5                        | 53.0            | 195                  |    |
| 2        | 0.53                   | 1.22                             | 74.0                            | 96.0                        | 48.8            | 189                  |    |
| 3        | 0                      | 0.79                             | 56.2                            | 68.0                        | 44.1            | 193                  |    |
| 4        | 0.55                   | 0.85                             | 58.1                            | 68.9                        | 50.7            | 192                  |    |
| 5        | 0.54                   | 0.96                             | 71.2                            | 90.0                        | 55.7            | 206                  |    |
| 6        | 0.94                   | 0.95                             | 89.2                            | 71.3                        | 47.6            | 214                  |    |
| 7        | 0.44                   | 0.76                             | 89.2                            | 65.8                        | 48.4            | 253                  |    |
| 8        | 0.39                   | 0.87                             | 89.4                            | 74.0                        | 50.8            | 258                  |    |
| 9        | 0.42                   | 0.74                             | 98.0                            | 66.5                        | 52.5            | 261                  | 30 |
| 10       | 0                      | 0.81                             | 70.1                            | 68.4                        | 42.1            | 210                  |    |
| 11       | 0                      | 0.91                             | 70.8                            | 76.0                        | 45.5            | 207                  |    |
| 12       | 0                      | 1.03                             | 70.0                            | 80.0                        | 44.4            | 185                  |    |
| 13       | 0.44                   | 0.85                             | 68.0                            | 72.2                        | 51.1            | 210                  |    |
| 14       | 0.47                   | 1.20                             | 97.0                            | 88.6                        | 50.1            | 193                  |    |

In the apparatus of Figures 6 and 7 at a steam temperature of about 2200° F., at an oxygen to coal ratio of about 32% and with the use of 0.6 pound of steam per pound of coal, the following results were obtained. At an oxygen concentration of 60%, 91% of the coal was gasified with a thermal efficiency of 55% to yield a gas having a heating value of 268 B. t. u. per cubic foot. At an oxygen concentration of 71%, 95% of the coal was gasified with a thermal efficiency of 65% to yield a gas having a heating value of 293 B. t. u. per cubic foot.

A rather significant fact is that the rate of nominal heat release was found to range around 500,000 B. t. u. per hour per cubic foot of the above-described apparatus at atmospheric pressure and a gas residence time of 0.3 second. This rate of heat release is as good or better than that secured in conventional carburetted water gas practice.

Many details of composition, procedure and structure may be varied within a wide range without departing from the principles of this invention, and it is, therefore, not our purpose to limit the patent granted on this invention otherwise than necessitated by a scope of the appended claims.

We claim:

1. A continuous method of gasifying coal at a high throughput rate which comprises suspending granular coal in a stream of flowing gas, passing said suspension through a restriction to produce an instantaneous pressure drop of at least 15 pounds per square inch to shatter the coal particles, immediately confining said suspension of shattered particles in a cylindrical, axially-limited space and incorporating therewith additional gas capable of reacting with the coal while forming said suspension into a vortex to completely intermix the reactants and further comminute said particles so that at least 80% will pass a 100 mesh screen and at least 50% will pass a 200 mesh screen, axially discharging continuously the comminuted particles from the center of said vortex into a reaction chamber, incorporating with said discharged suspension free oxygen-containing gas in an

amount sufficient to provide from 0.5 to 1.0 pound of total free oxygen per pound of coal to gasify the coal particles with the formation of ash, maintaining the temperature of said reaction chamber above the slagging temperature of the ash and separating the gas from the slag.

2. A continuous method of gasifying coal at a high throughput rate which comprises suspending granular coal in a stream of compressed gas, passing said suspension through a restriction to produce an instantaneous pressure drop of at least 15 pounds per square inch to shatter the coal particles, immediately confining said suspension of shattered particles in a cylindrical, axially-limited space maintained at elevated temperature and incorporating therewith oxygen-containing gas while forming said suspension into a vortex to completely intermix the reactants and further comminute said particles so that all will pass through a 100 mesh screen and at least 50% through a 325 mesh screen, axially discharging continuously the comminuted particles from the center of said vortex into a reaction chamber, incorporating with said discharged suspension additional oxygen-containing gas in an amount sufficient to provide 0.6 to 0.9 pound of total free oxygen per pound of coal to gasify the coal particles with the formation of ash, said oxygen-containing gas having at least 60% free oxygen, maintaining the temperature of said reaction chamber above the slagging temperature of the ash, and separating the gas from the slag.

3. A continuous method of gasifying coal at a high throughput rate which comprises suspending granular coal in a stream of compressed gas, passing said suspension through a restriction to produce an instantaneous pressure drop of at least 15 pounds per square inch to shatter the coal particles, immediately confining said suspension of shattered particles in a cylindrical, axially-limited space and incorporating therewith one-half to one pound of superheated steam per pound of coal while forming said suspension into a vortex to partially devolatilize and further comminute said particles so that all will pass through a 100 mesh screen and at least 50% through a 325 mesh screen, axially discharging continuously the comminuted particles from the center of said vortex into a reaction chamber, incorporating with said discharged suspension a free oxygen-containing gas in an amount sufficient to provide from 0.5 to 1 pound of total free oxygen per pound of coal to bring about complete gasification of the coal with the formation of ash, maintaining the temperature in said reaction chamber at least 2200° F. to bring about the blue gas reaction and to slag the ash, and discharging said gas from said reactor after a residence time therein of from 0.2 to 3.5 seconds.

4. A continuous method of gasifying coal at a high throughput rate which comprises suspending granular coal in a stream of compressed gas, passing said suspension through a restriction to produce an instantaneous pressure drop of at least 15 pounds per square inch to shatter the coal particles, introducing the flowing suspension of shattered particles into a stream of superheated steam confined within a cylindrical, axially-limited space to partially devolatilize and further comminute said particles so that all will pass through a 100 mesh screen and at least 50% will pass through a 325 mesh screen, the ratio of coal to steam being about 2 to 1 by weight, axially discharging continuously the comminuted particles from the center of said cylindrical space into a reaction chamber, incorporating with said discharged suspension a free oxygen-containing gas in an amount sufficient to provide from 0.5 to 1 pound of total free oxygen per pound of coal to bring about complete gasification of the coal with the formation of ash, maintaining the temperature in said reaction chamber at least 2200° F. to bring about the blue gas reaction and to slag the ash, and discharging said gas from said

reactor after a residence time therein of from 0.2 to 3.5 seconds.

5. The method of claim 1 in which said reaction chamber is maintained at superatmospheric pressure.

6. The method of claim 3 in which said reaction chamber is maintained at superatmospheric pressure. 5

**References Cited** in the file of this patent

UNITED STATES PATENTS

885,766 DeLaval ----- Apr. 28, 1908 10

|                 |       |               |
|-----------------|-------|---------------|
| Marconnet       | ----- | Dec. 8, 1908  |
| McDonald        | ----- | Aug. 8, 1939  |
| McDonald        | ----- | June 18, 1940 |
| Totzek          | ----- | Feb. 16, 1943 |
| Ramseyer et al. | ----- | Aug. 3, 1948  |
| Gaucher         | ----- | July 3, 1951  |
| Krejci          | ----- | July 29, 1952 |